



US006737017B2

(12) **United States Patent**  
Woodfield et al.

(10) **Patent No.:** US 6,737,017 B2  
(45) **Date of Patent:** May 18, 2004

(54) **METHOD FOR PREPARING METALLIC ALLOY ARTICLES WITHOUT MELTING**

(75) Inventors: **Andrew Philip Woodfield**, Madeira, OH (US); **Clifford Earl Shamblen**, Cincinnati, OH (US); **Eric Allen Ott**, Cincinnati, OH (US)

(73) Assignee: **General Electric Company**, Schenectady, NY (US)

(\*) Notice: Subject to any disclaimer, the term of this patent is extended or adjusted under 35 U.S.C. 154(b) by 0 days.

(21) Appl. No.: **10/172,217**

(22) Filed: **Jun. 14, 2002**

(65) **Prior Publication Data**

US 2003/0231974 A1 Dec. 18, 2003

(51) **Int. Cl.<sup>7</sup>** ..... **B22F 3/00**

(52) **U.S. Cl.** ..... **419/30**; 419/38; 75/351; 75/370; 75/371

(58) **Field of Search** ..... 419/30, 38; 75/351, 75/370, 371, 10.62

(56) **References Cited**

U.S. PATENT DOCUMENTS

2,799,570 A \* 7/1957 Reed et al. ..... 419/11  
2,828,199 A \* 3/1958 Findlay ..... 75/437  
4,373,947 A \* 2/1983 Buttner et al. ..... 75/228

4,525,206 A \* 6/1985 Soled et al. ..... 75/351  
4,687,632 A \* 8/1987 Hurd et al. ..... 419/45  
4,820,339 A \* 4/1989 Bienvenu et al. ..... 75/368  
5,032,176 A \* 7/1991 Kametani et al. ..... 75/416  
5,322,666 A 6/1994 Watwe ..... 419/32  
5,779,761 A 7/1998 Armstrong et al. ..... 75/370  
5,930,580 A 7/1999 Everett ..... 419/2  
5,958,106 A 9/1999 Armstrong et al. ..... 75/370  
6,540,811 B2 \* 4/2003 Hosoe et al. ..... 75/348  
6,582,651 B1 \* 6/2003 Cochran et al. ..... 419/5

FOREIGN PATENT DOCUMENTS

WO WO9964638 12/1999

\* cited by examiner

*Primary Examiner*—Ngoclan T. Mai

(74) *Attorney, Agent, or Firm*—Gregory O. Garmong; Kurt L. Ehresman; McNess Wallace & Nurick LLC

(57) **ABSTRACT**

An article of a base metal alloyed with an alloying element is prepared by mixing a chemically reducible nonmetallic base-metal precursor compound of a base metal and a chemically reducible nonmetallic alloying-element precursor compound of an alloying element to form a compound mixture. The alloying element is preferably thermophysically melt incompatible with the base metal. The method further includes chemically reducing the compound mixture to a metallic alloy, without melting the metallic alloy, and thereafter consolidating the metallic alloy to produce a consolidated metallic article, without melting the metallic alloy and without melting the consolidated metallic article.

**23 Claims, 2 Drawing Sheets**

FIG. 1



FIG. 3



FIG. 2

## METHOD FOR PREPARING METALLIC ALLOY ARTICLES WITHOUT MELTING

This invention relates to the preparation of metallic-alloy articles, such as titanium-alloy articles, without melting of the metallic alloy.

### BACKGROUND OF THE INVENTION

Metallic-alloy articles are fabricated by any of a number of techniques, as may be appropriate for the nature of the article. In one common approach, metal-containing ores are refined to produce a molten metal, which is thereafter cast. The ores of the metals are refined as necessary to remove or reduce the amounts of undesirable minor elements. The composition of the refined metal may also be modified by the addition of desirable alloying elements. These refining and alloying steps may be performed during the initial melting process or after solidification and remelting. After a metal of the desired composition is produced, it may be used in the as-cast form for some alloy compositions (i.e., cast alloys), or further worked to form the metal to the desired shape for other alloy compositions (i.e., wrought alloys). In either case, further processing such as heat treating, machining, surface coating, and the like may be utilized.

The production of metallic alloys may be complicated by the differences in the thermophysical properties of the metals being combined to produce the alloy. The interactions and reactions due to these thermophysical properties of the metals may cause undesired results. Titanium, a commercially important metal, in most cases must be melted in a vacuum because of its reactivity with the oxygen and nitrogen in the air. In the work leading to the present invention, the inventors have realized that the necessity to melt under a vacuum makes it difficult to utilize some desirable alloying elements due to their relative vapor pressures in a vacuum environment. The difference in the vapor pressures is one of the thermophysical properties that must be considered in alloying titanium. In other cases, the alloying elements may be thermophysically incompatible with the molten titanium because of other thermophysical characteristics such as melting points, densities, chemical reactivities, and tendency of strong beta stabilizers to segregate. Some of the incompatibilities may be overcome with the use of expensive master alloys, but this approach is not applicable in other cases.

There is therefore a need for an improved method to make alloys of titanium and other elements that present thermophysical melt incompatibilities. The present invention fulfills this need, and further provides related advantages.

### BRIEF SUMMARY OF THE INVENTION

The present invention provides a method for preparing an article made of an alloy of a metal such as titanium with a thermophysically melt-incompatible alloying element. The present approach circumvents problems which cannot be avoided in melting practice or are circumvented only with great difficulty and expense. The present approach permits a uniform alloy to be prepared without subjecting the constituents to the circumstance which leads to the incompatibility, specifically the melting process. Unintentional oxidation of the reactive metal and the alloying elements is also avoided. The present approach permits the preparation of articles with compositions that may not be otherwise readily prepared in commercial quantities. Master alloys are not used.

An article of a base metal alloyed with an alloying element is prepared by mixing a chemically reducible non-

metallic base-metal precursor compound of a base metal and a chemically reducible nonmetallic alloying-element precursor compound of an alloying element to form a compound mixture. The alloying element is preferably thermophysically melt incompatible with the base metal, but both thermophysically melt incompatible and thermophysically melt compatible alloying elements may be present. The method further includes chemically reducing the compound mixture to a metallic alloy, without melting the metallic alloy, and thereafter consolidating the metallic alloy to produce a consolidated metallic article, without melting the metallic alloy and without melting the consolidated metallic article.

The nonmetallic precursor compounds may be solid, liquid, or gaseous. The chemical reduction is preferably performed by solid-phase reduction, such as fused salt electrolysis of the precursor compounds in a finely divided solid form such as an oxide of the element; or by vapor-phase reduction, such as contacting vapor-phase halides of the base metal and the alloying element(s) with a liquid alkali metal or a liquid alkaline earth metal. The final article preferably has more titanium than any other element. The present approach is not limited to titanium-base alloys, however. Other alloys of current interest include aluminum-base alloys, iron-base alloys, nickel-base alloys, and magnesium-base alloys, but the approach is operable with any alloys for which the nonmetallic precursor compounds are available that can be reduced to the metallic state.

In another embodiment, a method for preparing an article made of titanium alloyed with an alloying element comprises the steps of providing a chemically reducible nonmetallic base-metal precursor compound of titanium base metal, and providing a chemically reducible nonmetallic alloying-element precursor compound of an alloying element that is thermophysically melt incompatible with the titanium base metal, and thereafter mixing the base-metal precursor compound and the alloying-element precursor compound to form a compound mixture. The method further includes chemically reducing the compound mixture to produce a metallic alloy, without melting the metallic alloy, and thereafter consolidating the metallic alloy to produce a consolidated metallic article, without melting the metallic alloy and without melting the consolidated metallic article. Other compatible features described herein may be used with this embodiment.

The thermophysical melt incompatibility of the alloying element with titanium or other base metal may be any of several types, and some examples follow. In the alloys, there may be one or more thermophysically melt incompatible elements, and one or more elements that are not thermophysically melt incompatible with the base metal.

One such thermophysical melt incompatibility is in the vapor pressure, as where the alloying element has an evaporation rate of greater than about 100 times that of titanium at a melt temperature, which is preferably a temperature just above the liquidus temperature of the alloy. Examples of such alloying elements include cadmium, zinc, bismuth, magnesium, and silver.

Another such thermophysical melt incompatibility occurs when the melting point of the alloying element is too high or too low to be compatible with that of titanium, as where the alloying element has a melting point different from (either greater than or less than) that of titanium of more than about 400° C. (720° F.). Examples of such alloying elements include tungsten, tantalum, molybdenum, magnesium, and tin. Some of these elements may be furnished in master

alloys whose melting points are closer to that of titanium, but the master alloys are often expensive.

Another such thermophysical melt incompatibility occurs when the density of the alloying element is so different from that of titanium that the alloying element physically separates in the melt, as where the alloying element has a density difference with titanium of greater than about 0.5 gram per cubic centimeter. Examples of such alloying elements include tungsten, tantalum, molybdenum, niobium, and aluminum.

Another such thermophysical melt incompatibility is where the alloying element, or a chemical compound formed between the alloying element and titanium, chemically reacts with titanium in the liquid phase. Examples of such alloying elements include oxygen, nitrogen, manganese, nickel, and palladium.

Another such thermophysical melt incompatibility is where the alloying element exhibits a miscibility gap with titanium in the liquid phase. Examples of such alloying elements include the rare earths or rare-earth-like elements such as cerium, gadolinium, lanthanum, erbium, yttrium, and neodymium.

Another, more complex thermophysical melt incompatibility involves the strong beta stabilizing elements that exhibit large liquidus-to-solidus gaps when alloyed with titanium. Some of these elements, such as iron, cobalt, chromium, nickel, or manganese, typically exhibit eutectic (or near-eutectic) phase reactions with titanium, and also usually exhibit a solid state-eutectoid decomposition of the beta phase into alpha phase plus a compound. Other such elements, such as bismuth and copper, typically exhibit peritectic phase reactions with titanium yielding beta phase from the liquid, and likewise usually exhibit a solid state eutectoid decomposition of the beta phase into alpha phase plus a compound. Such elements present extreme difficulties in achieving alloy homogeneity during solidification from melting. This results not only because of normal solidification partitioning causing micro-segregation, but also because melt process perturbations are known to cause separation of the beta-stabilizing-element-rich liquid during solidification to cause macro-segregation regions typically called beta flecks.

Another thermophysical melt incompatibility involves the alkali and alkali-earth metals, such as lithium and calcium, that typically have very limited solubility in titanium alloys. Finely divided dispersions of these elements, for example beta calcium in alpha titanium, may not be readily achieved using a melt process.

These and other types of thermophysical melt incompatibilities lead to difficulty or impossibility in forming acceptable alloys of these elements in a conventional melting practice. The present approach, in which the metals are not melted at all during production or processing, circumvents the thermophysical melt incompatibility to produce good quality, homogeneous alloys.

Some additional processing steps may be included in the present process. In some cases, it is preferred that the compound mixture be compacted, after the step of mixing and before the step of chemical reduction. The result is a compacted mass which, when chemically reduced, produces a spongy metallic material. After the chemical reduction step, the metallic alloy is consolidated to produce a consolidated metallic article, without melting the metallic alloy and without melting the consolidated metallic article. This consolidation may be performed with any physical form of the metallic alloy produced by the chemical reduction, but the

approach is particularly advantageously applied to consolidating of the pre-compacted sponge. Consolidation is preferably performed by hot pressing or hot isostatic pressing, extrusion, but without melting in each case. Solid state diffusion of the alloying elements may also be used to achieve the consolidation.

The consolidated metallic article may be used in the as-consolidated form. In appropriate circumstances, it may be formed to other shapes using known forming techniques such as rolling, forging, extrusion, and the like. It may also be post-processed by known techniques such as machining, heat treating, surface coating, and the like.

The present approach may be used to fabricate articles from the precursor compounds, entirely without melting. As a result, the characteristics of the alloying elements which lead to thermophysical melt incompatibility, such as excessive evaporation due to high vapor pressure, overly high or low melting point, overly high or low density, excessive chemical reactivity, strong segregation tendencies, and the presence of a miscibility gap, may still be present but cannot lead to inhomogeneities or defects in the final metallic alloy. The present approach thus produces the desired alloy composition of good quality, but without interference from these thermophysical melt incompatibilities that otherwise would prevent the formation of an acceptable alloy.

The present approach differs from prior approaches in that the metal is not melted on a gross scale. Melting and its associated processing such as casting are expensive and also produce some undesirably microstructures that either are unavoidable or can be altered only with additional expensive processing modifications. The present approach reduces cost and avoids structures and defects associated with melting and casting, to improve mechanical properties of the final metallic article. It also results in some cases in an improved ability to fabricate specialized shapes and forms more readily, and to inspect those articles more readily. Additional benefits are realized in relation to particular metallic alloy systems, for example the reduction of the alpha case defect for susceptible titanium alloys.

Several types of solid-state consolidation are known in the art. Examples include hot isostatic pressing, and pressing plus sintering, canning and extrusion, and forging. However, in all known instances these solid-state processing techniques start with metallic material which has been previously melted. The present approach starts with nonmetallic precursor compounds, reduces these precursor compounds to the initial metallic material, and consolidates the initial metallic material. There is no melting of the metallic form.

The preferred form of the present approach also has the advantage of being based in a powder-form precursor. Starting with a powder of the nonmetallic precursor compounds avoids a cast structure with its associated defects such as elemental segregation on a nonequilibrium microscopic and macroscopic level, a cast microstructure with a range of grain sizes and morphologies that must be homogenized in some manner for many applications, gas entrapment, and contamination. The present approach produces a uniform, fine-grained, homogeneous, pore-free, gas-pore-free, and low-contamination final product.

The fine-grain, colony-free structure of the initial metallic material provides an excellent starting point for subsequent consolidation and metalworking procedures such as forging, hot isostatic pressing, rolling and extrusion. Conventional cast starting material must be worked to modify and reduce the colony structure, and such working is not necessary with the present approach.

Another important benefit of the present approach is improved inspectability as compared with cast-and-wrought product. Large metallic articles used in fracture-critical applications are inspected multiple times during and at the conclusion of the fabrication processing. Cast-and-wrought product made of metals such as alpha-beta titanium alloys and used in critical applications such as gas turbine disks exhibit a high noise level in ultrasonic inspection due to the colony structure produced during the beta-to-alpha transition experienced when the casting or forging is cooled. The presence of the colony structure and its associated noise levels limits the ability to inspect for small defects to defects on the order of about  $\frac{1}{64}$ – $\frac{3}{64}$  of an inch in size in a standard flat-bottom hole detection procedure.

The articles produced by the present approach are free of the colony structure. As a result, they exhibit a significantly reduced noise level during ultrasonic inspection. Defects in the  $\frac{1}{64}$ , or less, of an inch range may therefore be detected. The reduction in size of defects that may be detected allows larger articles to be fabricated and inspected, thus permitting more economical fabrication procedures to be adopted, and/or the detection of smaller defects. For example, the limitations on the inspectability caused by the colony structure limit some articles made of alpha-beta titanium alloys to a maximum of about 10-inch diameter at intermediate stages of the processing. By reducing the noise associated with the inspection procedure, larger diameter intermediate-stage articles may be processed and inspected. Thus, for example, a 16-inch diameter intermediate-stage forging may be inspected and forged directly to the final part, rather than going through intermediate processing steps. Processing steps and costs are reduced, and there is greater confidence in the inspected quality of the final product.

The present approach is particularly advantageously applied to make titanium-base articles. The current production of titanium from its ores is an expensive, dirty, environmentally risky procedure which utilizes difficult-to-control, hazardous reactants and many processing steps. The present approach uses a single reduction step with relatively benign, liquid-phase fused salts or with liquid alkali metals. Additionally, alpha-beta titanium alloys made using conventional processing are potentially subject to defects such as alpha case, which are avoided by the present approach. The reduction in the cost of the final product achieved by the present approach also makes the lighter-weight titanium alloys more economically competitive with otherwise much cheaper materials such as steels in cost-driven applications.

Other features and advantages of the present invention will be apparent from the following more detailed description of the preferred embodiment, taken in conjunction with the accompanying drawings, which illustrate, by way of example, the principles of the invention. The scope of the invention is not, however, limited to this preferred embodiment.

#### BRIEF DESCRIPTION OF THE DRAWINGS

FIG. 1 is a perspective view of a metallic article prepared according to the present approach;

FIG. 2 is a block flow diagram of an approach for practicing the invention; and

FIG. 3 is a perspective view of a spongy mass of the initial metallic material.

#### DETAILED DESCRIPTION OF THE INVENTION

The present approach may be used to make a wide variety of metallic articles 20, such as a gas turbine compressor

blade 22 of FIG. 1. The compressor blade 22 includes an airfoil 24, an attachment 26 that is used to attach the structure to a compressor disk (not shown), and a platform 28 between the airfoil 24 and the attachment 26. The compressor blade 22 is only one example of the types of articles 20 that may be fabricated by the present approach. Some other examples include other gas turbine parts such as fan blades, fan disks, compressor disks, turbine blades, turbine disks, bearings, blisks, cases, and shafts, automobile parts, biomedical articles, and structural members such as airframe parts. There is no known limitation on the types of articles that may be made by this approach.

FIG. 2 illustrates a preferred approach for an article of a base metal and a thermophysically melt-incompatible alloying element. The method comprises providing a chemically reducible nonmetallic base-metal precursor compound, step 40, and providing a chemically reducible nonmetallic alloying-element precursor compound of an alloying element that is thermophysically melt incompatible with the base metal, step 42. "Nonmetallic precursor compounds" are nonmetallic compounds of the metals that eventually constitute the metallic article 20. Any operable nonmetallic precursor compounds may be used. Reducible oxides of the metals are the preferred nonmetallic precursor compounds in solid-phase reduction, but other types of nonmetallic compounds such as sulfides, carbides, halides, and nitrides are also operable. Reducible halides of the metals are the preferred nonmetallic precursor compounds in vapor-phase reduction. The base metal is a metal that is present in a greater percentage by weight than any other element in the alloy. The base-metal compound is present in an amount such that, after the chemical reduction to be described subsequently, there is more of the base metal present in the metallic alloy than any other element. In the preferred case, the base metal is titanium, and the base-metal compound is titanium oxide,  $TiO_2$  (for solid-phase reduction) or titanium tetrachloride (for vapor-phase reduction). The alloying element may be any element that is available in the chemically reducible form of the precursor compound. A few illustrative examples are cadmium, zinc, silver, iron, cobalt, chromium, bismuth, copper, tungsten, tantalum, molybdenum, aluminum, niobium, nickel, manganese, magnesium, lithium, beryllium, and the rare earths.

The nonmetallic precursor compounds are selected to provide the necessary metals in the final metallic article, and are mixed together in the proper proportions to yield the necessary proportions of these metals in the metallic article. For example, if the final article were to have particular proportions of titanium, aluminum, and vanadium in the ratio of 90:6:4 by weight, the nonmetallic precursor compounds are preferably titanium oxide, aluminum oxide, and vanadium oxide for solid-phase reduction, or titanium tetrachloride, aluminum chloride, and vanadium chloride for vapor-phase reduction. Nonmetallic precursor compounds that serve as a source of more than one of the metals in the final metallic article may also be used. These precursor compounds are furnished and mixed together in the correct proportions such that the ratio of titanium:aluminum:vanadium in the mixture of precursor compounds is that required in the metallic alloy that forms the final article (90:6:4 by weight in the example). In this example, the final metallic article is a titanium-base alloy, which has more titanium by weight than any other element.

The base-metal compound and the alloying compound are finely divided solids or gaseous in form to ensure that they are chemically reacted in the subsequent step. The finely divided base-metal compound and alloying compound may

be, for example, powders, granules, flakes, or the like. The preferred maximum dimension of the finely divided form is about 100 micrometers, although it is preferred that the maximum dimension be less than about 10 micrometers to ensure good reactivity.

The present approach is preferably, but not necessarily, utilized in conjunction with thermophysically melt incompatible alloys. "Thermophysical melt incompatibility" and related terms refer to the basic concept that any identified thermophysical property of an alloying element is sufficiently different from that of the base metal, in the preferred case titanium, to cause detrimental effects in the melted final product. These detrimental effects include phenomena such as chemical inhomogeneity (detrimental micro-segregation, macrosegregation such as beta flecks, and gross segregation from vaporization or immiscibility), inclusions of the alloying elements (such as high-density inclusions from elements such as tungsten, tantalum, molybdenum, and niobium), and the like. Thermophysical properties are intrinsic to the elements, and combinations of the elements which form alloys, and are typically envisioned using equilibrium phase diagrams, vapor pressure versus temperature curves, curves of densities as a function of crystal structure and temperature, and similar approaches. Although alloy systems may only approach predicted equilibrium, these envisioning data provide information sufficient to recognize and predict the cause of the detrimental effects as thermophysical melt incompatibilities. However, the ability to recognize and predict these detrimental effects as a result of the thermophysical melt incompatibility does not eliminate them. The present approach provides a technique to minimize and desirably avoid the detrimental effects by the elimination of melting in the preparation and processing of the alloy.

Thus, "thermophysical melt incompatible" and related terms mean that the alloying element or elements in the alloy to be produced do not form a well mixed, homogeneous alloy with the base metal in a production melting operation in a stable, controllable fashion. In some instances, a thermophysically melt incompatible alloying element cannot be readily incorporated into the alloy at any compositional level, and in other instances the alloying element can be incorporated at low levels but not at higher levels. For example, iron does not behave in a thermophysically melt incompatible manner when introduced at low levels, typically up to about 0.3 weight percent, and homogeneous titanium-iron-containing alloys of low iron contents may be prepared. However, if iron is introduced at higher levels into titanium, it tends to segregate strongly in the melt and thus behaves in a thermophysically melt incompatible manner so that homogeneous alloys can only be prepared with great difficulty. In other examples, when magnesium is added to a titanium melt in vacuum, the magnesium immediately begins to vaporize due to its low vapor pressure, and therefore the melting cannot be accomplished in a stable manner. Tungsten tends to segregate in a titanium melt due to its density difference with titanium, making the formation of a homogeneous titanium-tungsten alloy extremely difficult.

The thermophysical melt incompatibility of the alloying element with titanium or other base metal may be any of several types, and some examples follow.

One such thermophysical melt incompatibility is in the vapor pressure, as where the alloying element has an evaporation rate of greater than about 100 times that of titanium at a melt temperature, which is preferably a temperature just above the liquidus temperature of the alloy. Examples of

such alloying elements include cadmium, zinc, bismuth, magnesium, and silver. Where the vapor pressure of the alloying element is too high, it will preferentially evaporate, as indicated by the evaporation rate values, when co-melted with titanium under a vacuum in conventional melting practice. An alloy will be formed, but it is not stable during melting and continuously loses the alloying element so that the percentage of the alloying element in the final alloy is difficult to control. In the present approach, because there is no vacuum melting, the high melt vapor pressure of the alloying element is not a concern.

Another such thermophysical melt incompatibility occurs when the melting point of the alloying element is too high or too low to be compatible with that of titanium, as where the alloying element has a melting point different from (either greater than or less than) that of titanium of more than about 400° C. (720° F.). Examples of such alloying elements include tungsten, tantalum, molybdenum, magnesium, and tin. If the melting point of the alloying element is too high, it is difficult to melt and homogenize the alloying element into the titanium melt in conventional vacuum melting practice. The segregation of such alloying elements may result in the formation of high-density inclusions containing that element, for example tungsten, tantalum, or molybdenum inclusions. If the melting point of the alloying element is too low, it will likely have an excessively high vapor pressure at the temperature required to melt the titanium. In the present approach, because there is no vacuum melting, the overly high or low melting points are not a concern.

Another such thermophysical melt incompatibility occurs when the density of the alloying element is so different from that of titanium that the alloying element physically separates in the melt, as where the alloying element has a density difference with titanium of greater than about 0.5 gram per cubic centimeter. Examples of such alloying elements include tungsten, tantalum, molybdenum, niobium, and aluminum. In conventional melting practice, the overly high or low density leads to gravity-driven segregation of the alloying element. In the present approach, because there is no melting there can be no gravity-driven segregation.

Another such thermophysical melt incompatibility occurs when the alloying element chemically reacts with titanium in the liquid phase. Examples of such alloying elements include oxygen, nitrogen, silicon, boron, and beryllium. In conventional melting practice, the chemical reactivity of the alloying element with titanium leads to the formation of intermetallic compounds including titanium and the alloying element, and/or other deleterious phases in the melt, which are retained after the melt is solidified. These phases often have adverse effects on the properties of the final alloy. In the present approach, because the metals are not heated to the point where these reactions occur, the compounds are not formed.

Another such thermophysical melt incompatibility occurs when the alloying element exhibits a miscibility gap with titanium in the liquid phase. Examples of such alloying elements include the rare earths such as cerium, gadolinium, lanthanum, and neodymium. In conventional melting practice, a miscibility gap leads to a segregation of the melt into the compositions defined by the miscibility gap. The result is inhomogeneities in the melt, which are retained in the final solidified article. The inhomogeneities lead to variations in properties throughout the final article. In the present approach, because the elements are not melted, the miscibility gap is not a concern.

Another, more complex thermophysical melt incompatibility involves the strong beta stabilizing elements that

exhibit large liquidus-to-solidus gaps when alloyed with titanium. Some of these elements, such as iron, cobalt, and chromium, typically exhibit eutectic (or near-eutectic) phase reactions with titanium, and also usually exhibit a solid state-eutectoid decomposition of the beta phase into alpha phase plus a compound. Other such elements, such as bismuth and copper, typically exhibit peritectic phase reactions with titanium yielding beta phase from the liquid, and likewise usually exhibit a solid state eutectoid decomposition of the beta phase into alpha phase plus a compound. Such elements present extreme difficulties in achieving alloy homogeneity during solidification from the melt. This results not only because of normal solidification partitioning causing micro-segregation, but also because melt process perturbations are known to cause separation of the beta-stabilizing-element-rich liquid during solidification to cause macro-segregation regions typically called beta flecks.

Another thermophysical melt incompatibility involves elements such as the alkali metals and alkali-earth metals that have very limited solubility in titanium alloys. Examples include lithium and calcium. Finely divided dispersions of these elements, for example beta calcium in alpha titanium, may not be readily achieved using a melt process.

These and other types of thermophysical melt incompatibilities lead to difficulty or impossibility in forming acceptable alloys of these elements in conventional production vacuum melting. Their adverse effects are avoided in the present melt-less approach.

The base-metal compound and the alloying compound are mixed to form a uniform, homogeneous compound mixture, step 44. The mixing is performed by conventional procedures used to mix powders in other applications, for solid-phase reduction, or by the mixing of the vapors, for vapor-phase reduction.

Optionally, for solid-phase reduction of solid precursor compound powders the compound mixture is compacted to make a preform, step 46. This compaction is conducted by cold or hot pressing of the finely divided compounds, but not at such a high temperature that there is any melting of the compounds. The compacted shape may be sintered in the solid state to temporarily bind the particles together. The compacting desirably forms a shape similar to, but larger in dimensions than, the shape of the final article.

The mixture of nonmetallic precursor compounds is thereafter chemically reduced by any operable technique to produce an initial metallic material, without melting the initial metallic material, step 48. As used herein, "without melting", "no melting", and related concepts mean that the material is not macroscopically or grossly melted, so that it liquefies and loses its shape. There may be, for example, some minor amount of localized melting as low-melting-point elements melt and are diffusively alloyed with the higher-melting-point elements that do not melt. Even in such cases, the gross shape of the material remains unchanged.

In one approach, termed solid-phase reduction because the nonmetallic precursor compounds are furnished as solids, the chemical reduction may be performed by fused salt electrolysis. Fused salt electrolysis is a known technique that is described, for example, in published patent application WO 99/64638, whose disclosure is incorporated by reference in its entirety. Briefly, in fused salt electrolysis the mixture of nonmetallic precursor compounds is immersed in an electrolysis cell in a fused salt electrolyte such as a chloride salt at a temperature below the melting temperatures of the metals that form the nonmetallic precursor

compounds. The mixture of nonmetallic precursor compounds is made the cathode of the electrolysis cell, with an inert anode. The elements combined with the metals in the nonmetallic precursor compounds, such as oxygen in the preferred case of oxide nonmetallic precursor compounds, are removed from the mixture by chemical reduction (i.e., the reverse of chemical oxidation). The reaction is performed at an elevated temperature to accelerate the diffusion of the oxygen or other gas away from the cathode. The cathodic potential is controlled to ensure that the reduction of the nonmetallic precursor compounds will occur, rather than other possible chemical reactions such as the decomposition of the molten salt. The electrolyte is a salt, preferably a salt that is more stable than the equivalent salt of the metals being refined and ideally very stable to remove the oxygen or other gas to a low level. The chlorides and mixtures of chlorides of barium, calcium, cesium, lithium, strontium, and yttrium are preferred. The chemical reduction may be carried to completion, so that the nonmetallic precursor compounds are completely reduced. The chemical reduction may instead be partial, such that some nonmetallic precursor compounds remain.

In another approach, termed vapor-phase reduction because the nonmetallic precursor compounds are furnished as vapors or gaseous phase, the chemical reduction may be performed by reducing mixtures of halides of the base metal and the alloying elements using a liquid alkali metal or a liquid alkaline earth metal. For example, titanium tetrachloride and the chlorides of the alloying elements are provided as gases. A mixture of these gases in appropriate amounts is contacted to molten sodium, so that the metallic halides are reduced to the metallic form. The metallic alloy is separated from the sodium. This reduction is performed at temperatures below the melting point of the metallic alloy. The approach is described more fully in U.S. Pat. Nos. 5,779,761 and 5,958,106, whose disclosures are incorporated by reference.

The physical form of the initial metallic material at the completion of step 48 depends upon the physical form of the mixture of nonmetallic precursor compounds at the beginning of step 48. If the mixture of nonmetallic precursor compounds is free-flowing, finely divided particles, powders, granules, pieces, or the like, the initial metallic material is also in the same form, except that it is smaller in size and typically somewhat porous. If the mixture of nonmetallic precursor compounds is a compressed mass of the finely divided particles, powders, granules, pieces, or the like, then the final physical form of the initial metallic material is typically in the form of a somewhat porous metallic sponge 60, as shown in FIG. 3. The external dimensions of the metallic sponge are smaller than those of the compressed mass of the nonmetallic precursor compound due to the removal of the oxygen and/or other combined elements in the reduction step 48. If the mixture of nonmetallic precursor compounds is a vapor, then the final physical form of the initial metallic material is typically fine powder that may be further processed.

The chemical composition of the initial metallic alloy is determined by the types and amounts of the metals in the mixture of nonmetallic precursor compounds furnished in steps 40 and 42. The relative proportions of the metallic elements are determined by their respective ratios in the mixture of step 44 (not be the respective ratios of the compounds, but the respective ratios of the metallic element). In a case of interest, the initial metallic alloy has more titanium than any other element, producing a titanium-base initial metallic alloy.

The initial metallic alloy is in a form that is not structurally useful for most applications. Accordingly and preferably, the initial metallic alloy is thereafter consolidated to produce a consolidated metallic article, without melting the initial metallic alloy and without melting the consolidated metallic article, step 50. The consolidation removes porosity from the initial metallic alloy, desirably increasing its relative density to or near 100 percent. Any operable type of consolidation may be used. Preferably, the consolidation 50 is performed by hot isostatic pressing the initial metallic alloy under appropriate conditions of temperature and pressure, but at a temperature less than the melting points of the initial metallic alloy and the consolidated metallic article (which melting points are typically the same or very close together). Pressing, solid-state sintering, and canned extrusion may also be used, particularly where the initial metallic alloy is in the form of a powder. The consolidation reduces the external dimensions of the mass of initial metallic alloy, but such reduction in dimensions are predictable with experience for particular compositions. The consolidation processing 50 may also be used to achieve further alloying of the metallic article. For example, can used in hot isostatic pressing may not be evacuated so that there is a residual oxygen content. Upon heating for the hot isostatic pressing, the residual oxygen diffuses into and alloys with the titanium alloy.

The consolidated metallic article, such as that shown in FIG. 1, may be used in its as-consolidated form. Instead, in appropriate cases the consolidated metallic article may optionally be post processed, step 52. The post processing may include forming by any operable metallic forming process, as by forging, extrusion, rolling, and the like. Some metallic compositions are amenable to such forming operations, and others are not. The consolidated metallic article may also or instead be optionally post-processed by other conventional metal processing techniques in step 52. Such post-processing may include, for example, heat treating, surface coating, machining, and the like.

The metallic material is never heated above its melting point. Additionally, it may be maintained below specific temperatures that are themselves below the melting point. For example, when an alpha-beta titanium alloy is heated above the beta transus temperature, beta phase is formed. The beta phase transforms to alpha phase when the alloy is cooled below the beta transus temperature. For some applications, it is desirable that the metallic alloy not be heated to a temperature above the beta transus temperature. In this case care is taken that the alloy sponge or other metallic form is not heated above its beta transus temperature at any point during the processing. The result is a fine microstructure structure that is free of alpha-phase colonies and may be made superplastic more readily than a coarse microstructure. Because of the fine particle size resulting from this processing, less work is required to reach a fine structure in the final article, leading to a lower-cost product. Subsequent manufacturing operations are simplified because of the lower flow stress of the material, so that smaller, lower-cost forging presses and other metalworking machinery may be employed, and their is less wear on the machinery.

In other cases such as some airframe components and structures, it is desirably to heat the alloy above the beta transus and into the beta phase range, so that beta phase is produced and the toughness of the final product is improved. In this case, the metallic alloy may be heated to temperatures above the beta transus temperature during the processing, but in any case not above the melting point of the alloy.

When the article heated above the beta transus temperature is cooled again to temperatures below the beta transus temperature, a fine colony structure is formed that can inhibit ultrasonic inspection of the article. In that case, it 5 may be desirable for the article to be fabricated and ultrasonically inspected at low temperatures, without having been heated to temperatures above the beta transus temperature, so that it is in a colony free state. After completion of the ultrasonic inspection to verify that the article is defect-free, it may then be heat treated at a temperature above the beta transus temperature and cooled. The final article is less inspectable than the article which has not been heated above the beta transus, but the absence of defects has already been established.

The microstructural type, morphology, and scale of the article is determined by the starting materials and the processing. The grains of the articles produced by the present approach generally correspond to the morphology and size of the powder particles of the starting materials, when the solid-phase reduction technique is used. Thus, a 15 5-micrometer precursor particle size produces a final grain size on the order of about 5 micrometers. It is preferred for most applications that the grain size be less than about 10 micrometers, although the grain size may be as high as 100 micrometers or larger. As discussed earlier, the present approach avoids a coarse alpha-colony structure resulting from transformed coarse beta grains, which in conventional melt-based processing are produced when the melt cools into the beta region of the phase diagram. In the present approach, the metal is never melted and cooled from the melt into the beta region, so that the coarse beta grains never occur. Beta grains may be produced during subsequent processing as described above, but they are produced at 20 lower temperatures than the melting point and are therefore much finer than are beta grains resulting from cooling from the melt in conventional practice. In conventional melt-based practice, subsequent metalworking processes are designed to break up and globularize the coarse alpha structure associated with the colony structure. Such processing 25 is not required in the present approach because the structure as produced is fine and does not comprise alpha plates.

The present approach processes the mixture of nonmetallic precursor compounds to a finished metallic form without the metal of the finished metallic form ever being heated 30 above its melting point. Consequently, the process avoids the costs associated with melting operations, such as controlled-atmosphere or vacuum furnace costs in the case of titanium-base alloys. The microstructures associated with melting, typically large-grained structures, casting defects, and colony structures, are not found. Without such defects, the articles may be lighter in weight. In the case of susceptible titanium-base alloys, the incidence of alpha case formation is also reduced or avoided, because of the reducing 35 environment. Mechanical properties such as static strength and fatigue strength are improved.

The present approach processes the mixture of nonmetallic precursor compounds to a finished metallic form without the metal of the finished metallic form ever being heated 40 above its melting point. Consequently, the process avoids the costs associated with melting operations, such as controlled-atmosphere or vacuum furnace costs in the case of titanium-base alloys. The microstructures associated with melting, typically large-grained structures and casting 45 defects, are not found. Without such defects, the articles may be made lighter in weight because extra material introduced 50 to compensate for the defects may be eliminated. The greater 55

confidence in the defect-free state of the article, achieved with the better inspectability discussed above, also leads to a reduction in the extra material that must otherwise be present. In the case of susceptible titanium-base alloys, the incidence of alpha case formation is also reduced or avoided, because of the reducing environment.

Although a particular embodiment of the invention has been described in detail for purposes of illustration, various modifications and enhancements may be made without departing from the spirit and scope of the invention. Accordingly, the invention is not to be limited except as by the appended claims.

What is claimed is:

1. A method for preparing an article of a base metal alloyed with an alloying element, comprising the steps of
  - providing a chemically reducible nonmetallic base-metal precursor compound of a titanium base metal;
  - providing a chemically reducible nonmetallic alloying-element precursor compound of an alloying element; thereafter
  - mixing the base-metal precursor compound and the alloying-element precursor compound to form a compound mixture; thereafter
  - chemically reducing the compound mixture to a metallic alloy, without melting the metallic alloy; and thereafter
  - consolidating the metallic alloy to produce a consolidated metallic article, without melting the metallic alloy and without melting the consolidated metallic article.
2. The method of claim 1, wherein the step of providing the chemically reducible nonmetallic base-metal precursor compound includes the step of
  - providing the chemically reducible nonmetallic base-metal precursor compound in a finely divided solid form, and
  - wherein the step of providing the chemically reducible nonmetallic alloying-element precursor compound includes the step of
  - providing the chemically reducible nonmetallic alloying-element precursor compound in a finely divided solid form.
3. The method of claim 1, wherein the step of providing the chemically reducible nonmetallic base-metal precursor compound includes the step of
  - providing the chemically reducible nonmetallic base-metal precursor compound in a gaseous form, and
  - wherein the step of providing the chemically reducible nonmetallic alloying-element precursor compound includes the step of
  - providing a chemically reducible nonmetallic alloying-element precursor compound in a gaseous form.
4. The method of claim 1, wherein the step of providing a chemically reducible nonmetallic base-metal precursor compound includes the step of
  - providing a chemically reducible base-metal oxide.
  5. The method of claim 1, wherein the step of providing the chemically reducible nonmetallic alloying-element precursor compound includes the step of
    - providing the alloying-element precursor compound of the alloying element, wherein the alloying element is thermophysically melt incompatible with the base metal.
    6. The method of claim 1, wherein the step of providing the chemically reducible nonmetallic alloying-element precursor compound of the alloying element includes the step of

- providing a chemically reducible alloying-element oxide.
7. The method of claim 1, wherein the step of chemically reducing includes the step of
    - chemically reducing the compound mixture by solid-phase reduction.
    8. The method of claim 1, wherein the step of chemically reducing includes the step of
      - chemically reducing the compound mixture by fused salt electrolysis.
      9. The method of claim 1, wherein the step of chemically reducing includes the step of
        - chemically reducing the compound mixture by vapor-phase reduction.
      10. The method of claim 1, wherein the step of chemically reducing includes the step of
        - chemically reducing the compound mixture by contact with a liquid selected from the group consisting of a liquid alkali metal and a liquid alkaline earth metal.
      11. A method for preparing an article made of titanium alloyed with an alloying element, comprising the steps of
        - providing a chemically reducible nonmetallic base-metal precursor compound of titanium base metal;
        - providing a chemically reducible nonmetallic alloying-element precursor compound of an alloying element that is thermophysically melt incompatible with the titanium base metal; thereafter
        - mixing the base-metal precursor compound and the alloying-element precursor compound to form a compound mixture; thereafter
        - chemically reducing the compound mixture to produce a metallic alloy, without melting the metallic alloy; and thereafter
        - consolidating the metallic alloy to produce a consolidated metallic article, without melting the metallic alloy and without melting the consolidated metallic article.
      12. The method of claim 11, wherein the step of providing the chemically reducible nonmetallic alloying-element precursor compound of the alloying element includes the step of
        - providing the chemically reducible nonmetallic alloying-element precursor compound of the alloying element, wherein the alloying element has a vapor pressure of greater than about 100 times a vapor pressure of titanium in a titanium melt, both measured at a melt temperature.
        13. The method of claim 11, wherein the step of providing the chemically reducible nonmetallic alloying-element precursor compound of the alloying element includes the step of
          - providing the chemically reducible nonmetallic alloying-element precursor compound of the alloying element, wherein the alloying element has a melting point different from that of titanium by more than about 400° C.
        14. The method of claim 11, wherein the step of providing the chemically reducible nonmetallic alloying-element precursor compound of the alloying element includes the step of
          - providing the chemically reducible nonmetallic alloying-element precursor compound of the alloying element, wherein the alloying element has a density difference with titanium of greater than about 0.5 gram per cubic centimeter.
          15. The method of claim 11, wherein the step of providing the chemically reducible nonmetallic alloying-element precursor compound of the alloying element includes the step of

## 15

providing the chemically reducible nonmetallic alloying-element precursor compound of the alloying element, wherein the alloying element chemically reacts with titanium in a liquid phase to form chemical compounds including titanium and the alloying element.

16. The method of claim 11, wherein the step of providing the chemically reducible nonmetallic alloying-element precursor compound of the alloying element includes the step of

providing the chemically reducible nonmetallic alloying-element precursor compound of the alloying element, wherein the alloying element exhibits a miscibility gap with titanium in the liquid phase.

17. The method of claim 11, including an additional step, after the step of mixing and before the step of chemically reducing, of

compacting the compound mixture.

18. The method of claim 11, wherein the step of chemically reducing includes the step of

chemically reducing the compound mixture to produce the metallic alloy in the form of a sponge.

19. The method of claim 11, including an additional step, prior to the step of mixing, of

providing a chemically reducible nonmetallic alloying-element compatible precursor compound of an alloying element that is not thermophysically melt incompatible with the titanium base metal, and

wherein the step of mixing includes the step of

mixing the base-metal precursor compound, the alloying-element precursor compound, and the alloying-element compatible precursor compound to form a compound mixture.

20. A method for preparing an article of a base metal alloyed with an alloying element, comprising the steps of

providing a chemically reducible nonmetallic base-metal precursor compound of an aluminum base metal;

providing a chemically reducible nonmetallic alloying-element precursor compound of an alloying element; thereafter

mixing the base-metal precursor compound and the alloying-element precursor compound to form a compound mixture; thereafter

chemically reducing the compound mixture to a metallic alloy, without melting the metallic alloy; and thereafter

consolidating the metallic alloy to produce a consolidated metallic article, without melting the metallic alloy and without melting the consolidated metallic article.

21. A method for preparing an article of a base metal alloyed with an alloying element, comprising the steps of

## 16

providing a chemically reducible nonmetallic base-metal precursor compound of a nickel base metal;

providing a chemically reducible nonmetallic alloying-element precursor compound of an alloying element; thereafter

mixing the base-metal precursor compound and the alloying-element precursor compound to form a compound mixture; thereafter

chemically reducing the compound mixture to a metallic alloy, without melting the metallic alloy; and thereafter consolidating the metallic alloy to produce a consolidated metallic article, without melting the metallic alloy and without melting the consolidated metallic article.

22. A method for preparing an article of a base metal alloyed with an alloying element, comprising the steps of

providing a chemically reducible nonmetallic base-metal precursor compound of a magnesium base metal;

providing a chemically reducible nonmetallic alloying-element precursor compound of an alloying element; thereafter

mixing the base-metal precursor compound and the alloying-element precursor compound to form a compound mixture; thereafter

chemically reducing the compound mixture to a metallic alloy, without melting the metallic alloy; and thereafter consolidating the metallic alloy to produce a consolidated metallic article, without melting the metallic alloy and without melting the consolidated metallic article.

23. A method for preparing an article of a base metal alloyed with an alloying element, comprising the steps of

providing a chemically reducible nonmetallic base-metal precursor compound of an iron base metal;

providing a chemically reducible nonmetallic alloying-element precursor compound of an alloying element; thereafter

mixing the base-metal precursor compound and the alloying-element precursor compound to form a compound mixture; thereafter

chemically reducing the compound mixture to a metallic alloy by vapor phase reduction, without melting the metallic alloy; and thereafter

consolidating the metallic alloy to produce a consolidated metallic article, without melting the metallic alloy and without melting the consolidated metallic article.

\* \* \* \* \*

UNITED STATES PATENT AND TRADEMARK OFFICE  
**CERTIFICATE OF CORRECTION**

PATENT NO. : 6,737,017 B2

Page 1 of 1

DATED : May 18, 2004

INVENTOR(S) : Andrew Philip Woodfield, Clifford Earl Shamblen and Eric Allen Ott

It is certified that error appears in the above-identified patent and that said Letters Patent is hereby corrected as shown below:

Title page.

Item [74], *Attorney, Agent or Firm*, "McNess Wallace" should be -- McNees Wallace --.

Signed and Sealed this

Twenty-first Day of December, 2004

A handwritten signature in black ink, reading "Jon W. Dudas", is placed within a rectangular box with a dotted grid background.

JON W. DUDAS  
*Director of the United States Patent and Trademark Office*